

## UNITED STATES PATENT OFFICE

2,349,760

## ULTRAVIOLET-SENSITIVE PHOTOGRAPHIC ELEMENT

Earle E. Richardson and Jonas John Chechak,  
Rochester, N. Y., assignors to Eastman Kodak  
Company, Rochester, N. Y., a corporation of  
New Jersey

No Drawing. Application June 1, 1942,  
Serial No. 445,388

10 Claims. (Cl. 95—7)

This invention relates to a photographic element which is sensitive to the extreme ultraviolet portion of the spectrum.

In modern industrial and scientific research, spectrography plays a considerable part, and in this field the characteristics of various materials under the influence of ultraviolet radiations are of interest. Much of this kind of work is now done with the quartz spectrograph, and measurements are made from the visible as far to the ultraviolet as possible. This work is, of course, done with the help of commercially obtainable photographic plates or films. The materials available have, however, introduced defects due largely to the fact that the gelatin, in which the silver halide grains of the emulsion are embedded, absorbs the radiations of very short wavelengths, thereby preventing their action upon the silver halide grains, which in themselves are sensitive to the radiations.

A number of previous workers have attempted to overcome this drawback by incorporating in the emulsion a fluorescent substance. The purpose of such substances, in general, is to transform the radiations of short waves to radiations of longer wavelengths, which are not so strongly absorbed by the gelatin. In this way, the short wavelength radiation is changed to longer wavelength radiation, which is able to penetrate the gelatin and act upon the silver halide grains. These secondary radiations are usually of a blue or greenish color.

A method of sensitizing to the ultraviolet, which has advantages over the older method of incorporating the fluorescent material in the emulsion, consists of overcoating the emulsion with a thin film comprising ethyl-dihydro-collidine-carboxylate in order to bring about the necessary energy transformation. While the use of the collidine derivative necessitates no change in the developing and fixing procedure, it does require a wash with alcohol or a swabbing with cotton, while the element is in the developer. Other substances used in this connection may actually require removal by means of a suitable solvent before development of the photographic element.

We have now found an ultraviolet sensitizing layer which is completely removed in the regular alkaline developers and requires no additional treatment of any kind. After development the plate or film can be fixed in the usual manner, washed and dried. The materials which we employ to provide sensitivity to the ultraviolet are bis ammonium salts of aliphatic amines selected

from the group consisting of dialkyl and trialkyl amines in which each alkyl group contains from seven to twelve carbon atoms, and a bis sulfonic acid of the following general formula:



wherein R represents a member selected from the group consisting of amino, alkylamino and acylamino groups, and n represents a positive integer of from one to two. The bis ammonium salts obtained from the bis sulfonic acids containing acylamino groups are advantageously employed. These acylamino compounds are ordinarily crystalline substances which can be readily adapted to the practice of our invention. Typical examples of these bis ammonium salts are the bis diacetylamine salts of 4,4'-diacetylaminostilbene-2,2'-disulfonic acid; diacetyl-o-tolidine-2,2'-disulfonic acid and 4,4'-diacetylaminostilbene-2,2'-disulfonic acid.

To sensitize a photographic silver halide emulsion with our new ultraviolet sensitizers, the emulsion coated on a suitable support, such as a glass plate, is bathed for about thirty seconds in a 1% solution of the bis ammonium salt in ethyl alcohol. Following bathing, the excess solution is allowed to drain off and the photographic element is dried in a suitable position on a drying rack.

Our invention, of course, is directed primarily to the customarily employed gelatino silver chloride, chlorobromide, bromide and bromiodide developing-out emulsions. However, it can also be practiced with silver halide emulsions in which the carrier for the silver halide is other than gelatin, e. g. a cellulose derivative or a resin.

In addition to the bis ammonium salts recited above, we have found that the following bis ammonium salts are also efficacious ultraviolet sensitizers; the diacetylamine salts of 2-acetylaminonaphthalene-6,8-disulfonic acids and 1-acetylaminonaphthalene-6-sulfonic acid.

The bis ammonium salts which we employ in practicing our invention can be prepared as illustrated in the following example:

4,4' - diacetylaminostilbene - 2,2' - disulfonic acid  
bis-diacetylamine salt

30 g. of the sodium salt of 4,4'-diacetylaminostilbene-2,2'-disulfonic acid were dissolved in 600 cc. of water at 80° C. The hot solution was filtered and then cooled to 25° C. To the cooled solution was added slowly with stirring a solution

of 30 g. of diethylamine in 50 cc. of glacial acetic acid, 200 cc. of ethyl alcohol and 200 cc. of water. A white precipitate formed. The resulting mixture was stirred for one hour. The precipitate was then filtered off, washed with 500 cc. of cold water and pressed dry. The precipitate was dissolved in 500 cc. of boiling ethyl alcohol and the hot solution was filtered. The filtered solution was cooled somewhat and then poured slowly, with stirring, into 800 cc. of cold water. The bis diethylamine salt separated out as an oil which solidified and formed a powder after stirring for one hour. The resulting mixture was permitted to stand for several hours, after which the bis diethylamine salt was filtered off and washed with 500 cc. of cold water. The salt was pressed to remove water and was finally dried on the steam bath. Yield 45 g.

The other bis ammonium salts which we employ in practicing our invention can be similarly prepared, making due allowance for the molecular weight of the starting materials employed.

What we claim as our invention and desire to be secured by Letters Patent of the United States is:

1. A photo-sensitive silver halide emulsion containing a bis ammonium salt of an aliphatic amine and a bis sulfonic acid of the following general formula:



wherein  $n$  represents a positive integer of from one to two and R represents a member selected from the group consisting of amino, alkylamino and acylamino groups and Z represents a divalent organic radical, said aliphatic amine being selected from the group consisting of dialkyl and trialkyl amines in which each alkyl group contains from 7 to 12 carbon atoms.

2. A photo-sensitive gelatino silver halide emulsion containing a bis ammonium salt of an aliphatic amine and a bis sulfonic acid of the following general formula:



wherein  $n$  represents a positive integer of from one to two and R represents a member selected from the group consisting of amino, alkylamino and acylamino groups and Z represents a divalent organic radical, said aliphatic amine being selected from the group consisting of dialkyl and trialkyl amines in which each alkyl group contains from 7 to 12 carbon atoms.

3. A photo-sensitive gelatino silver halide developing-out emulsion containing a bis ammonium salt of an aliphatic amine and a bis sulfonic acid of the following general formula:



wherein  $n$  represents a positive integer of from one to two and R represents a member selected from the group consisting of amino, alkylamino and acylamino groups and Z represents a divalent organic radical, said aliphatic amine being selected from the group consisting of dialkyl and trialkyl amines in which each alkyl group contains from 7 to 12 carbon atoms.

4. A photo-sensitive silver halide emulsion containing a bis ammonium salt of an aliphatic amine and a bis sulfonic acid of the following general formula:



wherein  $n$  represents a positive integer of from one to two and R represents an acylamino group, and Z represents a divalent organic radical, said aliphatic amine being selected from the group consisting of dialkyl and trialkyl amines in which each alkyl group contains from 7 to 12 carbon atoms.

5. A photo-sensitive gelatino silver halide emulsion containing a bis ammonium salt of an aliphatic amine and a bis sulfonic acid of the following general formula:



wherein  $n$  represents a positive integer of from one to two and R represents an acylamino group, and Z represents a divalent organic radical, said aliphatic amine being selected from the group consisting of dialkyl and trialkyl amines in which each alkyl group contains from 7 to 12 carbon atoms.

6. A photo-sensitive gelatino silver halide developing-out emulsion containing a bis ammonium salt of an aliphatic amine and a bis sulfonic acid of the following general formula:



wherein  $n$  represents a positive integer of from one to two and R represents an acylamino group, and Z represents a divalent organic radical, said aliphatic amine being selected from the group consisting of dialkyl and trialkyl amines in which each alkyl group contains from 7 to 12 carbon atoms.

7. A photo-sensitive gelatino silver halide developing-out emulsion containing a bis ammonium salt of a diethyl amine and 4,4'-diacetyl-amino-stilbene-2,2'-disulfonic acid.

8. A photo-sensitive gelatino silver halide developing-out emulsion containing a bis ammonium salt of a diethyl amine and 4,4'-diacetyl-amino-dibenzyl-2,2'-disulfonic acid.

9. A photo-sensitive gelatino silver halide developing-out emulsion containing a bis ammonium salt of a diethyl amine and 4,4'-diacetyl-amino-diphenyl urea-3,3'-disulfonic acid.

10. A photo-sensitive gelatino silver halide developing-out emulsion containing a bis ammonium salt of a dialkyl amine and a bis sulfonic acid of the following general formula:



wherein R represents an acylamino group and Z represents a divalent organic radical, said dialkyl amine containing from 7 to 12 carbon atoms in each alkyl group.